

Patented June 5, 1928.

## UNITED STATES PATENT OFFICE.

JOHN WESLEY FRAZIER, OF SAN ANTONIO, TEXAS, ASSIGNOR TO UVALDE ROCK ASPHALT COMPANY, OF SAN ANTONIO, TEXAS.

## BITUMINOUS ROADWAY.

No Drawing.

Application filed April 15, 1924. Serial No. 706,741.

My invention relates to an improved method of constructing a base for roadways having a topping of bituminous material thereon.

5 It is an object of the invention to provide a method of forming a base for roadways which is firm and compact and capable of resisting the wear of traffic for long periods.

10 My road base is adapted to support a bituminous topping, preferably rock asphalt applied either hot or cold.

It is also desired to provide a roadway which is cheap to construct and economical to keep up.

15 It is particularly desired in the formation of my improvement to firmly bond the materials together so that they will not yield under loads and thus become uneven and rough.

20 In carrying out my invention I employ the usual mineral aggregate, which may be graded from pieces about 1 inch in thickness to broken particles of stone and sand of size small enough to pass through a 30

25 mesh screen. The material may be the usual crusher run of stone with the addition of sand, if necessary, to furnish enough fine materials to fill the voids between the larger particles.

30 The said mineral aggregate is run into a drum and heated thoroughly and an asphaltic base oil is added in the drum sufficient to thoroughly coat all the surface of the mineral particles. To accomplish this, 35 the drum is rotated and the temperature maintained so as to make the oil easily fluid.

The mineral particles when thus coated, adhere to the bituminous binder employed so that all the constituents become firmly 40 bonded together. The asphaltic oil being less viscous, can form a film thoroughly impregnating all the particles.

Pulverized rock asphalt is then added in the proportion of about 10% to 15% of the 45 mass. Said rock asphalt is taken in the form in which it comes from the quarry and is run through a rock crusher until it is reduced to a fine powder, containing particles ranging from  $\frac{1}{4}$  inch in thickness to 50 those which can pass through a 200 mesh

screen. It is then run into the drum and the drum rotated to thoroughly mix the coated mineral chips with the pulverized rock asphalt. The temperature of the charge is kept between 250° F. and 350° F. 55 for good results and should not be allowed to vary beyond these limits.

When the charge is thoroughly heated and mixed, it is discharged and distributed upon the sub grade. It is raked into a 60 smooth layer of the desired depth and rolled to solidly compact the mixture upon the roadway. A surfacing of richer material may be then added as desired, preferably 65 made up principally of pulverized rock asphalt thoroughly rolled and compacted.

I find, when a road surfacing is thus made and treated, the bituminous binder adheres firmly to the mineral particles so that the roadway becomes a solid mass which will 70 not break up or crack. The bituminous binder is sufficient to make the roadway flexible under the strains of traffic, temperature, and severe weather conditions.

The base thus formed is commonly called 75 black base and when constructed in the manner described, all the voids and interstices are filled with rock asphalt and said rock asphalt is thoroughly permeated with bitumen. The rock asphalt is much more effective in producing an efficient binder than is common asphalt in that the limestone is pure and is thoroughly impregnated with the heavy bitumen in a manner not possible to attain by artificial means. When finely 80 ground it may be compacted to form a homogeneous mass free of voids.

The proportions of materials may be varied somewhat depending on conditions 85 of traffic and the state of the sub grade upon 90 which the base is laid. I do not therefore desire to be limited to the exact proportions and form of the constituent parts.

What I claim as new, and desire to protect by Letters Patent is:

95 1. A process of forming bituminous road base comprising the heating of crushed rock and mineral particles, coating the same with a thin film of asphaltic oil, mixing therewith about 10% of the bulk in pulverized 100

rock asphalt, and agitating and mixing the same at a temperature of approximately 300° Fahrenheit.

2. A process of forming bituminous road base comprising the heating of crushed mineral aggregate, agitating the same and coating it with asphaltic oil, and mixing therewith about 10% of pulverized rock asphalt.

3. A process of forming bituminous road base comprising coating a charge of crushed mineral aggregate with asphaltic oil, and intimately mixing therewith about one tenth of the bulk in pulverized rock asphalt.

In testimony whereof I hereunto affix my signature this 5th day of April, A. D. 1924.

JOHN WESLEY FRAZIER.